

March 4, 1952

R. O'HALLORAN

2,588,279

LUBRICATING COMPOSITION

Filed Feb. 2, 1950



R. O'Halloran Inventor  
By *C. Wm. M. Thomas* Attorney

## UNITED STATES PATENT OFFICE

2,588,279

## LUBRICATING COMPOSITION

Rosemary O'Halloran, Elizabeth, N. J., assignor  
to Standard Oil Development Company, a cor-  
poration of Delaware

Application February 2, 1950, Serial No. 142,014

6 Claims. (Cl. 252—40)

1

This invention relates to a lubricating composition suitable for use as an all-purpose lubricant. More particularly, this invention relates to a lubricating grease which is compounded by blending separate grease components to form a grease having excellent lubricating properties at both high and low temperatures.

It is known in the art that grease compositions which are made by incorporating into a lubricating oil the desired amount of the sodium salt of a low molecular weight acid in addition to the sodium soap of a higher molecular weight fatty acid, have desirable properties that make them operable as lubricants for many purposes. For instance, these soda greases have excellent lubricating qualities at high temperatures and outstanding shear stability characteristics. Their dropping points are very high and they show excellent oxidation resistance and oil separation qualities. In some respects, however, these soda greases are undesirable for an all-purpose lubricant. The high soap content necessary to give them the desirable structural stability and shear breakdown resistance results in an excessively hard grease which does not soften when used for lubricating industrial machinery, resulting in undesirably noisy operation. At low temperatures, these soda greases fail to give satisfactory lubrication because of their high soap content and also because they can not be made using a lubricating oil having a low rate of viscosity change with temperature, a desirable dispersing medium for low temperature greases. Apparently the soap complex formed between the high and low molecular weight salts is excessively insoluble in a paraffinic mineral oil.

It is also known that greases prepared by dispersing a mixed soda-barium or soda-strontium soap of a high molecular weight fatty acid in a lubricating oil of high viscosity index, that is a viscosity index above about 75, have desirable low temperature lubrication characteristics and a soft structure which makes them of general use in industrial lubrication. These mixed soda-barium or soda-strontium soaps are easily dispersible in a lubricating oil having the desirable low rate of change of viscosity with temperature and thus have good lubricating properties at low temperatures. These mixed base greases, however, have the disadvantage of being only fair in structure stability generally and in some formulations having a relatively low dropping point.

It would be desirable to incorporate the advantages and properties of these two types of greases to obtain a soft, shear stable grease having a high dropping point, good oxidation stability and furnishing satisfactory lubrication at both high and low temperatures.

Attempts have been made to form such a grease by incorporating directly into a lubricating oil having a high viscosity index the desired amounts of the sodium and barium soaps of high molecular

2

weight fatty acids and a sodium salt of a low molecular weight organic acid. These attempts have failed, however, due to the coprecipitation of the high and low molecular weight soaps in the high viscosity index oil. This failure of dispersion is probably due to the incompatability of the complex soap containing low molecular weight organic acid salts and the high viscosity index oils at temperatures necessary for grease formation.

It has now been found and forms the subject of this invention that a grease composition incorporating the desirable characteristics of the soda greases and the mixed soda-barium greases may be made by a process of cold blending. Broadly speaking, the grease compositions of this invention are composed of two components. Component 1 is a soda-barium grease and component 2 is a grease containing the sodium soap of a high molecular weight substantially saturated fatty acid and the sodium salt of a low molecular weight organic acid. The two grease components are made separately and then blended together at room temperatures by the use of a suitable homogenizer or grease mill. It is felt that this successful blend is due to the similarity of the two component greases, both being substantially soda-soap-fatty acid greases. This is borne out by the fact that component 2 admixed with a calcium or lithium base grease results in a fluid mixture as does component 1 admixed with a soda-soap-rapeseed oil grease.

Component 1 may be described generally as being a grease formed by dispersing into a desirable lubricating oil a mixture of the sodium and barium soaps of any of the commonly known soap forming materials. The viscosity index of the oil chosen should be high enough to give the desired low temperature properties to the finished grease. Oils having a viscosity index above about 75 are especially desirable. A partial list of the soap forming materials would include hydrogenated fish oil acids, stearic acid, oleic acid, hydroxy stearic acid, beef fat, tallow, or mixtures of the above in any proportion. In the instant invention, the preferred embodiment contemplates a sodium-barium soap of hydrogenated fish oil acids.

The mol ratio of the sodium soap to the barium soap operable in the finished grease may vary from 1:1 to 25:1. The preferred ratio of sodium soap to barium soap is about 18:1. The amount of the mixture of soaps to be incorporated into the desired lubricating oil to form component 1 will depend upon the hardness of the final grease composition that is desired, since increasing the amount of soap in the grease increases the hardness of the composition. An operable range would be from 5% to 50% total soap content, 5% to 20% being preferred.

As to component 2, this ingredient is comprised of a mineral oil thickened to a grease consistency

with a mixture of a sodium soap of a high molecular weight fatty acid and a sodium salt of a low molecular weight organic acid. The sodium soap may be formed from any of the soap forming materials listed above, hydrogenated fish oil acids being again preferred. The low molecular weight organic acid to form the sodium salt may be selected from such acids as acetic, acrylic, furoic, or any of the other structure improving low molecular weight organic acids. In the preferred embodiment, sodium furoate is used.

The mol ratio of the sodium soap to the sodium salt may vary from 1:1 to 4:1 with mol ratios approaching 1:1 being preferred.

In blending the grease components of this invention, it is preferred to use from 90% to 65% of component 1 with 10% to 35% of component 2. Operable proportions, however, are from 95% to 50% of component 1 with 5% to 50% of component 2.

To illustrate more in detail the concept of this invention, the following example is given.

#### EXAMPLE I

##### Component 1

In a mineral oil blend having a viscosity index of 92 and a viscosity at 210° F. of 41.9 S. U. S. there was dispersed about 16.5% of a mixture of the sodium and barium soaps of a hydrogenated fish oil acid. The ratio of the sodium soap to the barium soap was 18:1. This grease was prepared in the usual manner by heating the ingredients to a temperature of about 400° F. and then pan-cooling the heated mixture to room temperature, followed by cold working of the grease cake to the desired penetration level.

##### Component 2

By the procedure described in a copending application, Serial No. 60,615, now United States Patent No. 2,516,137, issued July 25, 1950, a furfural grease was prepared by reacting 10% furfural into a furoic acid soap by the Cannizzaro reaction. This soap was combined with 15% of a sodium soap of hydrogenated fish oil acid and the mixture was added to a distillate having a viscosity index of about 60 and a viscosity at 210° F. of 36 S. U. S. The mixture of soap and oil was heated to a temperature of about 400° F. with stirring and was then pan-cooled to room temperature, followed by cold working.

##### Blend

75% of the soda barium grease and 25% of

the furfural grease was worked 5,000 strokes with the ASTM fine hole worker (325 holes  $\frac{1}{16}$ " in diameter). After this homogenization, a dark transparent grease of excellent appearance and structure resulted.

The properties of this cold blended grease in comparisons with component 1 alone are shown in Table I below:

TABLE I

|                                                                  | Properties of<br>Cold Blended<br>Grease | Sodium-<br>Barium<br>Base |
|------------------------------------------------------------------|-----------------------------------------|---------------------------|
| Penetration, mm./10, 60 strokes                                  | 288                                     | 295                       |
| Worked after 60,000 strokes (fine hole plate)                    | 286                                     | 359                       |
| ASTM Dropping Point, °F.                                         | 403                                     | 330                       |
| TORQUE @ -40° F. SEC./REV. (AN-G-15 Spec.)                       | 8.9                                     | 6.0                       |
| Oil Separation, Per Cent 50 Hrs./210° F.                         | 1.7                                     | 6.3                       |
| Water Wash, Per Cent Loss @ 77° F. (AN-G-5a Spec.)               | 0                                       | 0                         |
| Norma-Hoffman Oxidation Test, Hrs. to 5 p. s. i. Drop            | 500+                                    | 212                       |
| ABEC-NLG1 High Speed Spindle, Hrs. @ 250° F. and 10,000 R. P. M. | 675                                     | 549                       |

Inspection of the data set forth in Table I shows that the experimental grease blend has properties markedly superior to those of the sodium-barium grease which comprises 75% of the blend. The penetration of the blend has remained unchanged after long working, while that of the base softened 64 mm./10. The dropping point, oil separation, and Norma-Hoffman bomb oxidation are also improved. While the high speed spindle life of the grease at 250° F. is improved somewhat (23%) by the incorporation of the furoate grease, subsequent experimentation has shown that optimum spindle life is obtained with the use of lower amounts of the furoate grease, on the order of 10-15% of the total blend.

To show the utility of these new grease compositions in industrial usage various samples were prepared following generally the procedure of Example I. In these grease compositions, 75% of pan-cooled soda-barium greases of various soap contents in a 300 S. U. S./100° F. viscosity Coastal distillate were homogenized with 25% of a grease containing 23.2% sodium soaps. The sodium furoate (7%) was introduced into the grease as such or was produced in the grease by the Cannizzaro reaction. These different grades are shown containing 6%, 8% and 10% of the soda barium soap in component 1 and these products are compared with conventional soda-lime industrial greases containing 21% and 15% soap respectively.

TABLE II

## INDUSTRIAL GREASE BLENDS

## 75% Sodium/Barium Grease + 25% Sodium-Furoate Grease

| Soap Content Na/Ba<br>Base  | Total<br>Soap<br>Content,<br>Percent | Worked Penetration, mm./10 Fine<br>Hole Plate |                    |                     |                     | Drop<br>Point,<br>°F. | Oil Separa-<br>tion, percent<br>50/210° F. | Wheel<br>Bear-<br>ing<br>Test <sup>3</sup> | Percent<br>Loss<br>BEC<br>Test<br>@200° F. |
|-----------------------------|--------------------------------------|-----------------------------------------------|--------------------|---------------------|---------------------|-----------------------|--------------------------------------------|--------------------------------------------|--------------------------------------------|
|                             |                                      | 1,000 <sup>1</sup>                            | 5,000 <sup>1</sup> | 10,000 <sup>1</sup> | 10,000 <sup>2</sup> |                       |                                            |                                            |                                            |
| 6                           | 10.3                                 | 323                                           | 342                | 344                 | 349                 | 423                   | 10.0                                       | Pass                                       | 23                                         |
| 8                           | 11.8                                 | 294                                           | 317                | 318                 | 322                 | 417                   | 5.3                                        | do                                         | 13                                         |
| 10                          | 13.3                                 | 282                                           | 284                | 300                 | 301                 | 406                   | 3.6                                        | do                                         | 10                                         |
| Conventional Na/Ca Greases: |                                      |                                               |                    |                     |                     |                       |                                            |                                            |                                            |
| 21% Na/Ca Soap              |                                      | 326                                           | 375                |                     |                     | 350                   | 5.6                                        | Fail                                       | 73                                         |
| 13.5% Na/Ca Soap            |                                      | 420+                                          |                    |                     |                     | 345                   | 21.7                                       | do                                         |                                            |

<sup>1</sup> Penetration taken immediately after working.<sup>2</sup> Grease cooled 90 min., worked 60 strokes and repenetrated.<sup>3</sup> According to AXS-1574 Ford Wheel Bearing Test procedure.

It will be observed that the blended greases of this invention (although having considerably lower soap contents) show higher dropping points, better oil separation characteristics and better high temperature performance properties as measured by the wheel bearing test and the B. E. C. test than do the conventional industrial greases. Especially notable are the shear stability characteristics, the blend of greases breaking down only 20 to 30 penetration points during 10,000 strokes with the fine hole worker.

To obtain comparative data as to the pressure-viscosity relationship of the greases of this invention and the straight sodium-barium soap greases, the grease blend of Example I and component 11 were subjected to the standard pressure viscosity test. In this procedure, the greases were placed in a hydraulic-actuated grease cylinder fitted with an orifice calibrated to give a rate of shear of 100 sec.-1. The force required to maintain a constant rate of flow at different temperatures was recorded, the amount of force required being indicative primarily of the viscosity of the grease at the test temperature.

The accompanying drawing represents the pressure viscosity curves of these two greases and indicates their structural changes over a wide range of temperatures.

The observed changes in structure of the blend at temperatures in the neighborhood of 300° F. explain why the grease compositions of this invention can not be made by conventional methods. It is to be seen at temperatures below 300° F. the blended grease composition has a structure of essentially the same plasticity as the sodium-barium grease while showing improved properties of shear stability, oxidation resistance, oil separation, high temperature performance, etc. as discussed above. The sharp continued increase of the viscosity of the blended grease at temperatures in excess of 300° F. shows the incompatibility of the low molecular weight salt with the paraffinic mineral oil and depicts the undesirable thickening effect of the mixture. The change of structure of the blend at temperatures in the neighborhood of 300° F. may also be observed by the increasing amounts of hard granular undispersed material in the grease mixture. At temperatures in the neighborhood of 300° F. the high and low molecular weight soaps apparently form a complex which will not disperse in a paraffinic mineral oil having a high viscosity index.

The grease blends of this invention are perfectly compatible with the commonly used additive materials such as oxidation inhibitors, pour depressors, viscosity index improvers, anti-corrosion agents, and the like.

In summation, this invention is directed toward an improved lubricating composition which is capable of furnishing desirable lubrication properties at both high and low temperatures. It is also directed toward a method of incorporating into a paraffinic mineral oil having a low rate of change of viscosity with temperature, a salt of a low molecular weight organic acid. It is particularly concerned with an improved grease composition which comprises a blended grease formed from a sodium-barium grease and a sodium grease containing a sodium salt of a low molecular weight organic acid.

What is claimed is:

1. A blended grease composition which consists essentially of a mixture of two component greases, one component being from 95% to 50%

by weight based on the weight of the total composition of a grease formed from a mixture of the sodium and barium soaps of a high molecular weight substantially saturated fatty acid, the mol ratio of the sodium soap to the barium soap being from 1 to 1 to 25 to 1, and the other component being from 5% to 50% by weight based on the weight of the total composition of a grease formed from a mixture of the sodium soap of a high molecular weight substantially saturated fatty acid and the sodium salt of a low molecular weight organic carboxylic acid, the mol ratio of the soap and salt being from 1 to 1 to 4 to 1.

15 2. A blended grease composition which consists essentially of a blend of two component greases, one component being formed by dispersing in a paraffinic mineral oil having a high viscosity index a mixture of the sodium and barium soaps of a high molecular weight substantially saturated fatty acid, the mol ratio of said mixture of soaps being within a range of from 1:1 to 25:1 and the other component being a grease composition formed by dispersing in a mineral lubricating oil a sodium soap of a high molecular weight substantially saturated fatty acid and a sodium salt of a low molecular weight organic carboxylic acid, the mol ratio of the sodium soap to the sodium salt being within a range of from 1:1 to 4:1, said blend consisting essentially of from 90% to 65% by weight of the first component and from 10% to 35% by weight of the second component.

3. A grease composition according to claim 2 35 wherein the high molecular weight substantially saturated fatty acid is a hydrogenated fish oil acid and the sodium salt of the low molecular weight organic acid is sodium furoate.

4. A lubricating composition according to claim 2 40 wherein said first component consists essentially of from 5% to 50% of a mixture of sodium and barium soaps dispersed in a paraffinic type mineral oil, the ratio of said sodium soap to said barium soap being 18:1 to 8:1 and the mol ratio of the sodium soap to the sodium salt of said second component being within a range of from 4:1 to 1:1.

5. A method of preparing a lubricating grease composition having desirable lubricating characteristics at both high and low temperatures which comprises preforming a grease from a mixture of the sodium and barium soaps of a high molecular weight substantially saturated fatty acid, the mol ratio of the sodium soap to the barium soap being from 1 to 1 to 25 to 1, preforming a second grease composition from a mixture of the sodium soap of a high molecular weight substantially saturated fatty acid and the sodium salt of a low molecular weight organic carboxylic acid, and thereafter cold blending from 90% to 65% by weight of the first grease composition with from 10% to 35% by weight of the second grease composition.

6. A method of preparing a grease composition 65 having desirable lubricating characteristics at both high and low temperatures which comprises preforming a grease composition by dispersing in a mineral oil having a high viscosity index a mixture of the sodium and barium soaps of a high molecular weight substantially saturated fatty acid, the mol ratio of said sodium soap to said barium soap being within a range of from 1 to 1 to 25 to 1, preforming a second grease composition by dispersing in a mineral oil a mixture of the sodium soap of a high molecular weight sub-

7  
 substantially saturated fatty acid and a sodium salt of a low molecular weight organic carboxylic acid, the mol ratio of said soap to said salt being within a range of from 1 to 1 to 4 to 1 and thereafter cold blending from 90% to 65% by weight of the first grease composition with from 10% to 35% by weight of the second grease composition.

ROSEMARY O'HALLORAN.

REFERENCES CITED

10

UNITED STATES PATENTS

| Number    | Name          | Date          |
|-----------|---------------|---------------|
| 2,245,702 | Morway        | June 17, 1941 |
| 2,455,892 | Fraser        | Dec. 7, 1948  |
| 2,468,098 | Morway et al. | Apr. 26, 1949 |
| 2,468,099 | Morway        | Apr. 26, 1949 |
| 2,487,080 | Swenson       | Nov. 8, 1949  |
| 2,514,330 | Morway et al. | July 4, 1950  |
| 2,516,136 | Morway et al. | July 25, 1950 |
| 2,516,137 | Morway et al. | July 25, 1950 |
| 2,516,138 | Morway        | July 25, 1950 |

The following references are of record in the file of this patent: